

## UNITED STATES PATENT OFFICE

MICHAEL G. CORSON, OF JACKSON HEIGHTS, NEW YORK

## LEAD ALLOY AMENABLE TO HARDENING BY HEAT TREATMENT

No Drawing.

Application filed June 8, 1928. Serial No. 284,004.

It has within recent years been proposed to harden lead by adding to the lead anywhere from 1% to about 5% of antimony (the optimum being at 2.5%) and subjecting the alloy thus formed to heat treatment at 240° C. for about 30 minutes, this heat treatment being followed by quenching and aging. The theory of the process underlying the hardening of this alloy is based upon the

which would be precipitated in a lead alloy containing antimony and the second metal would consist of antimony atoms and atoms of the second metal in a definite proportion corresponding to the atomic proportions of such metals in their metallic compound, such particles would tend to grow only when they should happen to come together with antimony atoms and atoms of the second metal present in the solid solution of the lead in exactly the proportions such atoms bear towards one another in their metallic compound. As it is extremely improbable that atoms of the two metals will come together in precisely the proportions required to produce the definite compound of such metals, the tendency of the ultra-microscopic particles to grow will be substantially prevented.

10 assumption that antimony up to 2.5% stays in solid solution in lead at the temperature of heat treatment, remains so initially after quenching and is precipitated in an ultra-microscopic form during aging. These ultra-microscopic particles produce the slip interference effect and harden the alloy. Alloys of this character, as so far described in the literature and patented, suffer from the following drawbacks:

20 (1) The eutectic point of antimony—lead alloys is located at 243° C. Accordingly, the alloys cannot be heat treated at a higher temperature.

25 (2) The formation of the ultra-microscopic particles of antimony requires only the coming together in no definite proportion of the individual atoms of antimony, and the growth of these particles by the addition of other antimony atoms takes place whenever 30 any of such atoms and particles come together. Therefore, a further growth of these particles is continuously going on and both hardness and strength drop considerably in the course of time. For instance, an alloy 35 that shows a strength of 9800 lbs. per square inch on the tenth day of aging does not show more than 7500 lbs. after a few weeks have elapsed.

40 It has occurred to me that by substituting for the elementary antimony one of its metallic compounds, the second metal of this compound also being soluble to a substantial degree in solid lead, these two drawbacks might be eliminated due to the following reasons:

(1) The eutectic point would be raised, thereby permitting heat treatment at higher temperatures.

(2) Since the ultra-microscopic particles

Starting from this idea I have developed 70 alloys containing lead as a major component and cadmium in addition to antimony, the proportion of cadmium to antimony by weight ranging preferably from 1:1 to 3:2. I found that alloys of this kind have an 75 eutectic point approximately between 280 and 290° C. and, therefore, may be safely heat treated at 270 to 280° C. After this heat treatment has continued for about 1/2 hour to 1 hour the alloys may be either 80 quenched in water and aged or allowed to cool in air. Both methods lead to the same type of hardening and very high strength figures (8700 lbs. per square inch yield point and 10,800 lbs. per square inch tensile strength) 85 are obtained at the end of the first three hours. These figures increase further in a slow way only and become 9000 lbs. yield point and 11,700 lbs. strength after two days. The storing of these alloys does not undermine 90 their properties, i. e., does not weaken them in any degree.

The alloys may contain from 0.5% to 15% cadmium and from 0.5% to 15% antimony. At the lower contents of both additional 95 metals I obtain alloys which are easily rolled into sheet, drawn into wire, extruded into tubes, etc. With the higher amounts of both metals I obtain alloys which have a structure very desirable from the viewpoint of a 100

bearing metal. In this connection, I am aware of the fact that the presently used lead base bearing alloys containing antimony or antimony plus tin develop primary crystals of either antimony or a tin-antimony compound, which latter act as the hard constituent in the soft matrix. These constituents are however, specifically much lighter than lead and tend to segregate. In 10 my alloys the hard constituent or the cadmium-antimony compound is also much lighter than lead but shows however a tendency to crystallize in such a manner as to form cellular aggregates, with the surrounding lead eutectic. Therefore, they remain very evenly distributed through the whole alloy.

When an alloy capable of being rolled or otherwise worked is desired, it is preferred 20 to maintain the proportion of antimony between 0.5 and 5% and that of cadmium between 0.5 and 5%. An alloy combining the highest strength with a sufficient elongation of any thus produced by me contained about 25 1% cadmium and about 1% antimony. I have found that the ductility of the alloy decreases with the increase of antimony above 1%. On the other hand, increase of the amount of cadmium does not have much 30 influence on ductility unless such increase is accompanied by decrease of the amount of antimony to less than 1%, in which event the strength drops and the elongation increases.

35 A number of tests of lead alloys containing antimony and cadmium within the range specified, and rolled into sheet form, heat treated and aged according to the method above outlined, has shown the following 40 average properties for the product:

Tensile strength.....11,000 lbs./sq. in.  
Yield point.....8,900 lbs./sq. in.  
Elongation in 2".....12.5%  
Area reduction.....25.0%  
45 Brinell # (1/16" ball).  
(2 kgs. load).....27.0

When the alloy contains from 5 to 15% each of cadmium and antimony a material 50 suitable as a bearing metal in the cast state with or without heat treatment is produced. As an example, an alloy containing 10% cadmium and 12% antimony showed as cast a tensile strength of 9,500 lbs. per square inch 55 and a Brinell hardness of 24.0. The hardness of this alloy may be increased by applying heat treatment similar to the method above outlined.

While it is preferred to heat treat the lead- 60 antimony-cadmium alloys of the present invention between 270° and 280° C., it will be understood that the desired effects may be produced by heating at lower temperatures down to 200° C.

65 It is understood that various modifications

in the proportions of the various metals in the alloys may be made, and that various details of the method of heat treating may be modified without departing from the scope of the invention which is not to be deemed as limited other than as indicated in the appended claims.

What I claim is:

1. A method of hardening an alloy consisting principally of lead, and containing 75 0.5 to 15% each of antimony and cadmium, which comprises heating said alloy to a temperature upwards of 200° C. and short of the melting point for a sufficient period of time to bring the antimony and cadmium into solid solution in the lead matrix and then cooling to produce supersaturation followed by aging.

2. A method of hardening an alloy consisting principally of lead, and containing 85 0.5 to 15% each of antimony and cadmium, which comprises heating said alloy at from 270° to 280° C. for at least 30 minutes, and thereafter quenching to produce supersaturation followed by aging.

3. A hardened and worked metal article 90 consisting principally of lead and containing approximately 1% each of antimony and cadmium, and characterized by a physical structure and properties such as are produced when an alloy of like composition is subjected to heat treatment at such a temperature and for such time as to bring the antimony and cadmium into solid solution in the lead, followed by cooling to produce 100 supersaturation and then by aging.

4. A hardened and worked metal article 105 consisting principally of lead and containing 0.5% to 5% each of antimony and cadmium, and characterized by a physical structure and properties such as are produced when an alloy of like composition is subjected to heat treatment at such a temperature and for such time as to bring the antimony and cadmium into solid solution in the lead, followed by cooling to produce 110 supersaturation and then by aging.

In testimony whereof, I have signed my name to this specification this 4th day of June, 1928.

MICHAEL G. CORSON.